

# UNITED STATES PATENT OFFICE.

REUBEN C. RUTHERFORD, OF NEW YORK, N. Y.

## METHOD OF RESTORING FULLED WOOLEN FABRICS TO THEIR ORIGINAL DIMENSIONS.

SPECIFICATION forming part of Letters Patent No. 398,847, dated March 5, 1889.

Application filed September 28, 1887. Serial No. 250,906. (No specimens.)

*To all whom it may concern:*

Be it known that I, REUBEN C. RUTHERFORD, of the city, county, and State of New York, have invented a new and Improved Method 5 of Restoring Fullled Woolen Fabrics to Their Original Dimensions, of which the following is a full, clear, and exact description.

The object of my invention is to restore shrunken or fullled woolen fabrics to their 10 original dimensions and texture.

It is well known that the value of woven, knit, or felted woolen fabrics is greatly affected by their liability to full or shrink when saturated with moisture, and that this shrink- 15 age is greatly exaggerated by manipulation—increasing the thickness of the fabric and reducing its other dimensions. My improved process is designed to restore fullled goods of this description to their original dimensions,

20 or, if desirable, to increase their length and width at the expense of the thickness. The surface of the woolen fibers is in the form of imbricated scales, acting like barbs in the movement of the fibers upon one another.

25 The fibers are also wavy or kinky, the finer grades tending to the spiral form. Shrinkage is due to one or both of these factors—the scales and kinks. Moisture or manipulation (especially both) contracts the kinks and 30 moves the fibers readily in the direction of the base of their scales, which interlock to prevent movement in the opposite direction. Experiment shows that brief exposure of woolen fiber to the action of steam or water at the 35 boiling-point has no injurious effect upon the fiber or fabric. It is well known that the temperature of unconfined steam cannot be raised above that of the boiling-point of water. Exposed to the action of steam or water heated to 40 the boiling-point all keratinous substances—as horn, hoof, hair, and wool—become soft, yielding, and plastic. Thus heated by unconfined steam, the softened fibers may be straightened by tension, the resistance of the 45 interlocked scales (or barbs) overcome and bent back, thus permitting the fibers to slip upon one another, and so increasing their united length. Distention of the fabric at too low a temperature (which must be within its 50 elastic limit or result in rupture) is followed by partial or complete recoil. Distention under the other conditions described above is

permanent till the fabric is again subjected to the fulling or shrinking influences, when it will contract as before, showing that the integrity of the fabric and fiber remains intact under the process. In fact, the fabric is softer, smoother, more silky in appearance, and just as pliable and elastic as before the treatment.

55 In carrying out my invention I submit the fullled goods to a moist heat at or above the boiling-point of water, at the same time stretching the goods in the direction required to restore them to their original dimensions. The very high temperature softens the fibers of the wool, so that as the garment or piece is stretched the kinks and imbrications of the wool fibers readily slip past each other and allow the fabric to be stretched, and the fabric after this treatment will remain in its extended condition.

60 The following is a description of my method in detail: The garment is drawn over a wire frame adjustable to the required lateral dimensions of the part to be treated. This is 65 laid upon a board or table covered with a porous fabric—felt or cloth—which readily permits the passage of steam through its meshes. A well-moistened cotton or linen cloth is laid 70 smoothly upon the woolen fabric, and over this a highly-heated smoothing-iron is briskly passed, forcing the steam through the woolen fabric into the cloth beneath. While thus heated the part is stretched to the required 75 length with perfect ease. The dampened cloth 80 is then removed, and the woolen fabric, still held in position, ironed dry with an iron not hot enough to scorch the woolen. If the garment is shrunk laterally as well as longitudinally, the lateral dimension should be first 85 restored and retained in that position by the frame while stretching in the other direction. It is observed that in this way both sides of the garment treated are stretched and ironed 90 at once and in less time than in the ordinary 95 laundering.

100 In carrying out my invention upon a large scale I place the fabrics upon suitable adjustable stretching-frames and expose them to the action of steam of a sufficiently high temperature to soften the fibers above described, and after stretching them to the required dimensions I remove the fabrics from the steam and allow them to dry, or iron them

till dry with an iron that will not scorch the woolen fiber if a smooth or silky surface is desired.

Having thus fully described my invention, 5 I claim as new and desire to secure by Letters Patent—

1. The method of restoring fulled woolen fabrics to their original dimensions, which consists in stretching the fabric while subjected to moist heat at a temperature of about 10  $212^{\circ}$  Fahrenheit, substantially as specified.

2. The herein-described method of restoring shrunken woolen fabric, which consists in first exposing the fabric to the action of steam to 15 soften the fibers, then stretching the steamed fabric to the desired extent while it is in a

moist and heated condition, and finally drying the steamed and stretched fabric, substantially as set forth.

3. The herein-described method of restoring 20 shrunken woolen fabric, which consists in first forcing steam through the fabric, then stretching the steamed fabric to the desired extent while it is in a moist and heated condition, and then subjecting the stretched and steamed 25 fabric to a hot ironing to dry it, substantially as set forth.

REUBEN C. RUTHERFORD.

Witnesses:

GEO. M. HOPKINS,  
C. SEDGWICK.